

## UNITED STATES PATENT OFFICE

1,937,844

PHOTOGRAPHIC DEVELOPER AND METHOD  
OF DEVELOPINGMarion C. Reed, Charleston, W. Va., assignor to  
The B. F. Goodrich Company, New York, N. Y.,  
a corporation of New YorkNo Drawing. Application March 23, 1931  
Serial No. 524,759

14 Claims. (Cl. 95—88)

This invention relates to the art of photography, and particularly to the development of latent images in silver halide photographic emulsions.

5 It has been the general practice to develop silver halide photographic emulsions such as those on the familiar dry plates, photographic films, bromide and gas-light papers, etc., by immersing them in a mildly alkaline solution of an organic  
10 reducing agent such as hydroquinone, pyrogallol, monomethyl p-aminophenol, glycine, etc. The chief object of this invention, then, is to provide a new class of developing agents which exhibit certain distinct advantages over the previously  
15 known developers. Another object is to provide a class of developers which are far less expensive than the ones which are now in common use. Other objects will be evident from the following description of the invention.

20 The new developers which are employed in accordance with this invention are members of a class of substances having the general formula

25



where the dotted line indicates the atoms required to complete the heterocyclic ring, R is an aromatic nucleus, and X is a reducing grouping such as a hydroxyl or amino group. The preferred members of the class are compounds in which the heterocyclic ring contains an oxygen or sulphur atom and in which X is a hydroxyl group, such as the hydroxy-aryl morpholines.

30 The following substances, for example, are typical members of the class described above: p-hydroxy N-phenyl morpholine, m-methyl p-hydroxy N-phenyl morpholine, m-methoxy p-hydroxy N-phenyl morpholine, m-hydroxy N-phenyl morpholine, o-hydroxy N-phenyl morpholine, hydroxy N-naphthyl morpholine, hydroxy N-biphenyl morpholine, dihydroxy N-phenyl morpholine, amino hydroxy N-phenyl morpholine, ethylamino  
40 hydroxy N-phenyl morpholine, hydroxy N-phenyl thiomorpholine, hydroxy N-phenyl piperidine, p, p'-dihydroxy, N, N'-diphenyl piperazine, hydroxy 1,4 phenylene dimorpholine, hydroxy N-phenyl pyrrole, hydroxy N-phenyl tetra-hydro pyrrole,  
45 hydroxy N-phenyl hydroxyquinoline, p-amino N-phenyl morpholine, diamino N-phenyl morpholine, monomethyl diamino N-phenyl morpholine, etc.

50 The new developers of the class described above  
55 may be used for the development of photographic

images in the ordinary manner, preferably in a weakly alkaline solution. They possess a higher molecular weight than most of the previously known developers, hence somewhat greater proportions may be required, but this necessity is offset by the lower cost of many of these new developers and the superior results attained by their use.

55 As a specific example of one embodiment of this invention, a developing solution is prepared containing as developer m-methyl p-hydroxy N-phenyl morpholine



70

according to the following formula:

|                  | Parts |
|------------------|-------|
| Sodium sulphite  | 3     |
| Developer        | 7     |
| Sodium carbonate | 6     |
| Water            | 1000  |

80 Plates or films which have been given a normal exposure to light are developed by immersion in the solution for from 15 to 25 minutes at a temperature of about 18° C. (65° F.). They are then washed, fixed in a solution of sodium hyposulphite and washed thoroughly, in the usual manner. The photographic reproductions obtained by this 85 process are soft and pleasing, the details being well brought out by the action of the developer, while at the same time the contrast is good and sharp and the whites are clear. The new developer allows an unusual latitude in the degree of 90 exposure, good results being obtained even with emulsions which are somewhat under or over-exposed.

95 The new developers of this invention are admirably adapted for tank development, because of their tendency to correct the effects of improper exposure. They are particularly desirable for landscape or portrait work where the ability to reproduce detail is of greater importance than the production of the utmost degree of contrast. 100 They may be kept in stock almost indefinitely, either dry or in the form of a solution, for they are far more stable than the majority of the developers now in common use, and do not deteriorate on standing, even in moderately strong sun- 105 light.

110 Although a specific embodiment of the invention has been described with considerable particularity, it is to be understood that this invention is not limited thereby, but that it is sus-

ceptible of numerous variations within the scope of the appended claims, as will be obvious to those skilled in the art. In particular, the new developers of this invention may be used in conjunction with other known developers, or with other salts, acids or alkalies to modify the properties of the developing solution or of the photographic images obtained thereby. Such modifications are well known expedients and need not be described here.

This invention is a continuation in part of my copending application Serial No. 442,043, filed April 5, 1930.

I claim:

15. 1. A photographic developer comprising a solution of a compound having the structural formula



where the dotted line indicates the atoms required to complete the heterocyclic ring, R is an aromatic nucleus, and X is a hydroxyl or amino group.

25. 2. A photographic developer comprising a solution of a compound having the structural formula



35. 3. where the dotted line indicates the atoms required to complete a six-membered, saturated, heterocyclic ring, and R is an aromatic nucleus.

40. 4. A photographic developer comprising a solution of a hydroxy N-aryl morpholine in which the aryl group contains only one aromatic ring.

45. 5. A photographic developer comprising a solution of a p-hydroxy N-aryl morpholine in which the aryl group contains only one aromatic ring.

6. A photographic developer comprising a solution of m-methyl p-hydroxy N-phenyl morpholine.

50. 7. A photographic developer comprising a dilute aqueous solution of a hydroxy N-aryl morpholine.

55. 8. A photographic developer comprising a dilute alkaline aqueous solution of a hydroxy N-aryl morpholine.

9. A process of developing photographic images which comprises treating a silver halide photographic emulsion which has been exposed to the light with a compound having the structural formula

80



where the dotted line indicates the atoms required to complete the heterocyclic ring, R is an aromatic nucleus, and X is a hydroxyl or amino group.

10. A process of developing photographic images which comprises immersing a silver halide photographic emulsion which has been exposed to the light in a solution comprising a compound having the structural formula

90



where the dotted line indicates the atoms required to complete a six-membered, saturated, heterocyclic ring, and R is an aromatic nucleus.

11. A process of developing photographic images which comprises immersing a silver halide photographic emulsion which has been exposed to the light in an aqueous solution comprising a hydroxy N-aryl morpholine.

105

12. A process of developing photographic images which comprises immersing a silver halide photographic emulsion which has been exposed to the light in an aqueous solution comprising a hydroxy N-aryl morpholine in which the aryl group contains only one aromatic ring.

110

13. A process of developing photographic images which comprises immersing a silver halide photographic emulsion which has been exposed to the light in a dilute, aqueous, alkaline solution comprising a p-hydroxy N-aryl morpholine in which the aryl group contains only one aromatic ring.

115

14. A process of developing photographic images which comprises immersing a silver halide photographic emulsion which has been exposed to the light in an aqueous, alkaline solution comprising m-methyl p-hydroxy N-phenyl morpholine.

120

MARION C. REED.

130

60

135

65

140

70

145

75

150